

May 20, 1958

L. E. THIESS

2,835,019

METHOD FOR CASTING CERAMIC SHAPES

Filed Sept. 12, 1955



*Fig. 3.*

Inventor  
Ludwig E. Thiess,  
by Gilbert P. Tarleton  
His Attorney.

1

2,835,019

## METHOD FOR CASTING CERAMIC SHAPES

Ludwig E. Thiess, Baltimore, Md., assignor to General Electric Company, a corporation of New York

Application September 12, 1955, Serial No. 533,688

2 Claims. (Cl. 25—156)

This invention relates to the manufacture of ceramic members, and more particularly, to a method for casting ceramic shapes.

In the prior art it is well known to form relatively large porcelain bushings by a casting process utilizing an upright porous mold having a cavity therein complementary to the configuration of the porcelain bushing. Conventionally, a hose of casting slip is directed into the upper end of the cavity to fill same. Inasmuch as the casting slip enters the cavity on one side the casting slip flows in two paths from said one side to the opposite side of the cavity. These two flows of the casting slip meet at said opposite side and form what is known in the art as a slip meeting mark. This slip meeting mark usually is a dark brown or black wide streak adjacent the bottom of the cast bushing which ends in a dark vertical line higher up in the bushing.

A study of the nature of this discolored area has shown that it consists essentially of suspended organic matter having been introduced by the dark, fine, lignite particle containing ball-clays of alkaline casting slip. Apparently, this colloidal organic matter and the colloidal clay fractions, being lighter in weight, segregate from the liquid slip and are carried to the surface where the slip meets in the mold, and there they produce a structural weakness or dividing line which is a source of cracks in the ware during drying and firing.

It is very difficult to avoid the formation of slip meeting marks in casting articles from ceramic casting slips. For instance, it has been observed that if the slip is poured into the mold from two opposite places two slip meeting lines will be formed. Additionally, experiments whereby the mold was filled from the bottom instead of the top have also not been entirely successful in eliminating slip meeting lines and weak areas.

In filling such molds it is also important that air entrapment in the cast piece be avoided. Such air may be present in the ceramic slip, but more often it is introduced into the cast insulator shapes by splashing of the slip in the mold or by filling the molds faster than the air can be safely displaced from the mold cavity.

Accordingly, it is an object of this invention to provide a method for casting ceramic shapes whereby slip meeting marks and entrapped air are eliminated.

I have discovered that rotary stirring of the slip as it rises in the mold will to a considerable degree eliminate slip meeting marks.

Additionally, the slip must be so poured into the mold cavity as to enable air present in the slip to be able to free itself, and the pouring must be controlled and at a predetermined rate to avoid splashing and to avoid filling the mold cavity faster than air can be safely displaced from the mold cavity.

My invention comprises a method of casting a hollow ceramic shape in a mold having a casting cavity therein for forming said ceramic shape, said method including pouring a stream of ceramic casting slip into said cavity

2

and simultaneously moving said stream about said cavity during said pouring.

My invention further comprises a method of casting a hollow elongated ceramic shape in a mold having a generally upright casting cavity therein for forming said ceramic shape, said method including controlled pouring of a downwardly directed stream of ceramic casting slip into said cavity along the inner surface of said cavity at an acute angle at a predetermined rate of flow and simultaneous moving of said stream around said cavity along said inner surface during said pouring at a predetermined rate of travel.

The features of my invention which I believe to be novel are set forth with particularity in the appended claims. My invention itself, however, both as to its organization and method of operation, together with further objects and advantages thereof, may best be understood by reference to the following description taken in connection with the accompanying drawing.

20 In the drawing, Fig. 1 is a partly broken away elevation view of one form of my invention. Fig. 2 is a partly broken away sectional view of my invention taken along the line 2—2 of Fig. 1. Fig. 3 is a partly broken away elevation view of a finished insulator similar to that illustrated as being formed in Fig. 1. Like reference numerals will be used throughout the various figures to indicate like parts.

Referring now particularly to Fig. 1, shown therein is a generally upright porous mold, such as a plaster of Paris mold, having a generally annular elongated upright casting cavity 1 therein. The mold cavity 1 is defined by a tapered central core section 2 and two mating generally conical hollow outer mold halves 3 which are banded together by bands 4 and concentrically spaced from central core section 2. The porous mold is used to manufacture by casting a high voltage porcelain insulator bushing of the type shown in Fig. 3 and having a plurality of petticoats 5 thereon.

40 The bottom of the mold is closed by a base sealing plate 6, and positioned on the top of the mold is a pouring and stirring tripod apparatus. The pouring and stirring apparatus comprises a vertical tubular member 7 aligned with the axis of cavity 1 and rotatably mounted in a stationary hub member 8. The hub 8 is mounted in spaced relationship with respect to the upper end of the mold by virtue of at least three adjustable legs 9 whose radial spread with respect to the axis of tube 7 can be adjusted by virtue of sleeves 10 and set screws 11.

45 Mounted on the hub 8 is a support bracket 12 which supports an adjustable speed drive motor 13 whose shaft carries a small gear 14. Small gear 14 engages and drives a large gear 15 which is coupled to the tube 7 whereby rotary motion is imparted to tube 7. The upper end of the tube 7 has a funnel 16 attached thereto adapted to receive ceramic casting slip from an inlet pipe 17 having a valve 18 therein. The lower end of the tube 7 has a generally crank-shaped outlet pipe 19 connected thereto and the lower end of pipe 19 is fitted with a nozzle 20 according to the rate of slip flow desired.

It will be noted that the outer surface of the core section 2 has a conical taper imparted thereto which is narrowest at the upper end thereof and widest at the lower end thereof. The radial distance of the nozzle 20 from the axis of tube 7 is selected so that the downwardly directed stream 21 of the casting slip will approach the tapered surface of core section 2 at an acute angle and run down the tapered surface of core section 2. This gives any air present in the slip an opportunity to free itself and also avoids splashing of the slip. The nozzle 20 is selected so as to give a rate of slip flow or rate of slip rise in the mold cavity 1 whereby air in the cavity 1

proper and in the petticoat cavities 5' have sufficient opportunity to escape before filling.

While the stream 21 is being poured the motor 13 due to gears 14 and 15 causes the stream 21 to continuously move around or about the annular outline of the cavity 1 at a relatively slow speed along the tapered surface of core section 2. Such rotary stirring of the slip by rotary feeding of the stream 21 I have discovered eliminates slip meeting marks which will result from stationary hose feeding. For an insulator approximately 3 feet high having an inner and outer diameter of about 6 and 12 inches respectively 4 to 6 revolutions per minute of the stream 21 and a rate of flow of about 1 cubic foot per minute have proven satisfactory. It will be obvious that the number of revolutions per minute of the stream 21 and the rate of flow of the slip will vary according to the size and configuration of the insulator being cast. However, a slow rate of flow is selected so that at least several passes of the stream around the mold are required to fill the same, and the speed of travel of the stream around the mold is slow so as to avoid centrifugal separation of the ingredients of the casting slip. For the same reason the mold is stationary. That is, high speed rotation of the stream or rotation of the mold causes centrifugal segregation of the slip ingredients which will result in a cast piece which is mechanically and electrically unsound.

In actual practice the funnel 16 can be made large enough to prohibit spilling over of the slip from the funnel 16 even though the valve 18 is fully opened. Initial pouring of the slip into the funnel 16 I have found to be useful since air present in the slip has an opportunity to escape therefrom while in the funnel 16.

As will be obvious to those skilled in the art, after the mold cavity 1 is completely filled it is allowed to stand so as the porous mold can absorb moisture from the casting slip. After the casting slip has set sufficiently and shrunk from the interior surfaces of the porous mold the bands 4 can be removed, the two mold halves 3 opened, and the set ceramic shape lifted or otherwise removed from about the core section 2.

While there has been shown and described a particular embodiment of the invention, it will be obvious to those skilled in the art that changes and modifications may be

made without departing from the invention, and therefore it is intended by the appended claims to cover all such changes and modifications as fall within the true spirit and scope of the invention.

5 What I claim as new and desire to secure by Letters Patent of the United States is:

1. In a method of forming large elongated cylindrical ceramic electrical insulating bushings by casting, the improvement of filling an upright mold having a large elongated cylindrical casting cavity without the formation of slip meeting marks, said improvement comprising pouring a stream of ceramic casting slip into the upper end of said mold and simultaneously rotating said stream about said mold while said mold is stationary, said stream having a rate of travel about said mold which is insufficient to cause centrifugal separation of the ingredients of said casting slip and requiring at least several passes about said mold to fill the same.
2. In a method of forming large elongated cylindrical ceramic electrical insulating bushings by casting, the improvement of slowly filling an upright mold having a large elongated cylindrical casting cavity without the formation of slip meeting marks in the piece to be cast, said improvement comprising directing a downward stream of ceramic casting slip into the upper end of said mold at an acute angle against an interior surface of said mold and simultaneously slowly rotating said stream around said mold while said mold is stationary, said stream having a low rate of flow and requiring several passes around said mold to fill the same, and said stream being rotated around said mold at a slow speed to avoid centrifugal segregation of the ingredients of said casting slip.

References Cited in the file of this patent

| UNITED STATES PATENTS |               |               |
|-----------------------|---------------|---------------|
| 35 1,304,571          | Kirk et al.   | May 27, 1919  |
| 1,885,774             | Showers       | Nov. 1, 1932  |
| 2,026,624             | Flower        | Jan. 7, 1936  |
| FOREIGN PATENTS       |               |               |
| 40 745,431            | France        | Feb. 14, 1933 |
| 652,418               | Great Britain | Apr. 25, 1951 |